

# United States Patent [19]

Lauterbach-Dammler

[11] 3,925,261

[45] Dec. 9, 1975

[54] **EXPONENTIAL RESISTANCE MATERIAL AND METHOD OF MANUFACTURING SAME**

[75] Inventor: **Inge Lauterbach-Dammler, Nurnberg, Germany**

[73] Assignee: **C. Conradty, Nurnberg, Germany**

[22] Filed: **July 16, 1974**

[21] Appl. No.: **489,182**

[30] **Foreign Application Priority Data**

July 18, 1973 Germany..... 2336504

[52] **U.S. Cl.** ..... **252/519; 252/518; 252/520; 264/61; 264/67; 264/104**

[51] **Int. Cl.<sup>2</sup>** ..... **H01B 1/08**

[58] **Field of Search** ..... **252/518-521; 264/67, 61, 104**

[56] **References Cited**

UNITED STATES PATENTS

3,642,664 2/1972 Masuyama et al..... 252/519  
3,658,725 4/1972 Masuyama et al..... 252/519 X

*Primary Examiner*—Benjamin R. Padgett

*Assistant Examiner*—E. Suzanne Parr

*Attorney, Agent, or Firm*—Gifford, Chandler & Sheridan

[57]

## ABSTRACT

A voltage drop across a resistance element, wherein the resistance varies exponentially with the voltage, is expressed by the equation:

$$E = B \times I^n$$

wherein  $I$  is the current through the element,  $B$  is a constant and is equal to the voltage value at which the current through the element is equal to 1 Ampere, and  $E$  is the voltage drop. To achieve a variable B-value based on the resistance material itself and furthermore to achieve a greater dependence of the resistance on the voltage drop, the value of  $n$  can be selectively raised by varying the composition of the resistance element as follows:

50 – 90% ZnO  
0.1 – 40% ZnF<sub>2</sub>  
0.1 – 40% MeO

wherein MeO is an oxide selected from the oxides of magnesium, calcium, strontium, barium, iron, cobalt, lead, boron, aluminum, bismuth, manganese, chromium, nickel, antimony, and mixtures thereof. An improved method of manufacturing such a resistance material is also described.

**10 Claims, No Drawings**

## EXPONENTIAL RESISTANCE MATERIAL AND METHOD OF MANUFACTURING SAME

### BACKGROUND OF THE INVENTION

The invention relates to a resistance material wherein the resistance varies exponentially with the voltage drop and, more particularly, relates to a sintered ceramic material for non-linear resistance elements. The invention also relates to a method of manufacturing such material.

Such resistance materials are well known and have been made from, for example, silicon carbide, titanium dioxide or zinc oxide. The voltage drop across elements made from such materials is given by the following equation:

$$E = B \times I^{1/n}$$

wherein  $E$  is the voltage drop over the element,  $I$  is the current flowing through the element, and  $B$  is a constant reflecting the voltage value at current  $I = 1$  Ampere. The exponent  $n$  is, therefore, a direct measure of the magnitude of non-linearity based on p-n-transitions, on the contact among the individual grains, or on the material itself.

It is known that the  $B$ -value of a non-linear resistance element may be varied by sintering at varying temperatures and under different atmospheres. It is further known to adjust the  $B$ -value through the thickness of the resistance elements. Both procedures permit only a limited possibility of variation. Thus, when there is a change in temperature the desired  $n$ -value, in many cases, is not attained and when there is a change in thickness, desired small increments of resistance often are not attainable.

### DESCRIPTION OF THE INVENTION

It is therefore an object underlying the invention to provide a composition wherein the electrical resistance is greatly dependent on voltage and thus has a large  $n$ -value and a variable  $B$ -value based on the material itself.

It is a further object to provide a method of manufacturing such a composition.

The first object is particularly advantageously solved by a composition comprising about 50-90%  $ZnO$ , about 0.1 - 40%  $ZnF_2$ , and about 0.1 - 40%  $MeO$ ; wherein  $MeO$  is an oxide selected from the oxides of magnesium, calcium, strontium, barium, iron, cobalt, lead, boron, aluminum, bismuth, manganese, chromium, nickel, antimony, and mixtures thereof. According to the invention, the  $B$ -value of the material may be varied within wide ranges by changing the ratio of the two components  $ZnO$  and  $ZnF_2$ . If, meanwhile, the metal oxide content is kept unchanged, the  $n$ -value of the material remains nearly constant. However the  $n$ -value can be adjusted to many values by varying the  $MeO$  content.

The following Examples and the Table explain in more detail the relationship of the electric properties of the compositions of the invention and the method of manufacture of the compositions.

### EXAMPLE 1

Two mole % each of  $Bi_2O_3$ ,  $Co_3O_4$ ,  $MnO_2$  and  $Sb_2O_3$  (a preferred composition) were homogeneously mixed with varying amounts of  $ZnO$  and  $ZnF_2$ . After a presintering at 600°C the material was ground, compacted to

a selected shape, and annealed at 1000° to 1400°C. Electrical contacts were made on the ends of the resulting elements by flame-spraying with brass and, in some cases, by coating with conductive silver. Optionally, 5 terminal wires (pigtails) can be attached.

As can be seen from the values in Table 1, the  $B$ -value increases nearly linearly with increasing  $ZnF_2$  content, whereas the  $n$ -value of 20 to 25 remains nearly constant.

### EXAMPLE 2

Three mole % of each of  $Bi_2O_3$ ,  $Co_3O_4$ ,  $MnO_2$  and  $Sb_2O_3$  were homogeneously mixed together with varying amounts of  $ZnO$  and  $ZnF_2$  and were further processed according to the procedure described in Example 1.

The electrical values of the resulting element are listed in Table 1 (numbers 7-9). A comparison with Examples 1 to 6 shows that a small change in the metal oxide content effects a considerable change in the  $n$ -value.

TABLE 1

| No. | ZnO/ZnF <sub>2</sub><br>(mole%) | Bi <sub>2</sub> O <sub>3</sub> | Co <sub>3</sub> O <sub>4</sub> | MnO <sub>2</sub><br>(mole %) | Sb <sub>2</sub> O <sub>3</sub> | B<br>(Volts at<br>1 mA) | n  |
|-----|---------------------------------|--------------------------------|--------------------------------|------------------------------|--------------------------------|-------------------------|----|
| 1   | 92/0.1                          | 2                              | 2                              | 2                            | 2                              | 196                     | 22 |
| 2   | 90/2                            | 2                              | 2                              | 2                            | 2                              | 226                     | 20 |
| 3   | 88/4                            | 2                              | 2                              | 2                            | 2                              | 255                     | 20 |
| 4   | 84/8                            | 2                              | 2                              | 2                            | 2                              | 337                     | 24 |
| 5   | 76/16                           | 2                              | 2                              | 2                            | 2                              | 413                     | 25 |
| 6   | 60/32                           | 2                              | 2                              | 2                            | 2                              | >1000                   |    |
| 7   | 87/1                            | 3                              | 3                              | 3                            | 3                              | 273                     | 43 |
| 8   | 86/2                            | 3                              | 3                              | 3                            | 3                              | 285                     | 41 |
| 9   | 85/3                            | 3                              | 3                              | 3                            | 3                              | 313                     | 40 |

Repetition of the foregoing examples with a wide variety of compositions having differing  $ZnO$  to  $ZnF_2$  ratios and differing proportions of the oxides of the invention established that the advantages of the invention were attained when the  $ZnO$  was in the range of about 50-90%, the  $ZnF_2$  was in the range of about 0.1 - 40%, and the  $MeO$  was in the range of about 0.1 - 40%. Further, the composition was found to be particularly useful when the  $ZnF_2$  content was about 1-8% and the  $MeO$  content was about 2-16%.

Similarly, repetition of the above examples with presintering at various temperatures and annealing the formed element at various temperatures showed that the best forming conditions for the resistance material was presintering at about 600°-900°C and annealing at about 1000°-1400°C.

It is, of course, to be understood that the present invention is not limited to the specific examples given, but also comprises any modifications within the scope of the appended claims.

I claim:

1. A composition adapted for use as an electrical resistance element wherein the electrical resistance varies exponentially with the voltage drop across the element, said voltage drop being given by the equation:

$$E = B \times I^{1/n}$$

wherein  $E$  is said voltage drop;  $I$  is the current through the element,  $B$  is a constant equal to the voltage value at which the current is equal to 1 Ampere, and  $n$  is a number; said composition comprising about 50-90%  $ZnO$ , about 0.1 - 40%  $ZnF_2$ , and about 0.1 - 40%  $MeO$ ; wherein  $MeO$  is an oxide selected from the oxides of magnesium, calcium, strontium, barium, iron, cobalt, lead, boron, aluminum, bismuth, manganese, chro-

mium, nickel, antimony, and mixtures thereof.

mium, nickel, antimony, and mixtures thereof.

2. The composition according to claim 1 in which the  $ZnF_2$  proportion is about 1-8% and the MeO content is about 2-16%.

3. The composition according to claim 1 wherein said MeO is approximately equal molar proportions of  $Bi_2O_3$ ,  $Co_3O_4$ ,  $MnO_2$ , and  $Sb_2O_3$ .

4. The composition according to claim 2 wherein said MeO is approximately equal molar proportions of  $Bi_2O_3$ ,  $Co_3O_4$ ,  $MnO_2$ , and  $Sb_2O_3$ .

5. The composition according to claim 1 wherein said composition is in the form of a resistance element.

6. The method of manufacturing a composition adaptable for use as an electrical resistance element which method comprises the steps of

a. forming a homogeneous mixture of about 50-90%  $ZnO$ , about 0.1 - 40%  $ZnF_2$ , and about 0.1 - 40% MeO wherein MeO is an oxide selected from the oxides of magnesium, calcium, strontium, barium, iron, cobalt, lead, boron, aluminum, bismuth, man-

ganese, chromium, nickel, antimony, and mixtures thereof;

b. sintering said mixture at about 600°-900°C.;

c. grinding the sintered mixture;

d. compacting the resulting mixture; and

e. annealing the resulting material at about 1000° - 1400°C.

10. The method according to claim 6 wherein said ground mixture is compacted to the form of a resistance element.

8. The method according to claim 6 wherein said MeO is approximately equal molar proportions of  $Bi_2O_3$ ,  $Co_3O_4$ ,  $MnO_2$ , and  $Sb_2O_3$ .

9. The method according to claim 7 wherein said MeO is approximately equal molar proportions of  $Bi_2O_3$ ,  $Co_3O_4$ ,  $MnO_2$ , and  $Sb_2O_3$ .

10. The method according to claim 6 and further comprising the step of positioning metal electrical contacts on portions of said resistance element.

\* \* \* \* \*

25

30

35

40

45

50

55

60

65